

# UNITED STATES PATENT OFFICE.

GEORGE ATKINS, OF SHARON, PENNSYLVANIA, ASSIGNOR TO HIMSELF,  
GEORGE W. WESTERMAN, ROBERT FOX, ROBERT MAY, AND SAMUEL  
T. ATKINS, OF SAME PLACE.

## IMPROVEMENT IN THE MANUFACTURE OF SHEET-IRON.

Specification forming part of Letters Patent No. 88,002, dated March 23, 1869.

Be it known that I, GEORGE ATKINS, of the town of Sharon, county of Mercer, and State of Pennsylvania, have invented a new and useful Process for the Manufacture of Sheet-Iron, by which I produce an article superior to anything now publicly known and used, which shall possess much of the appearance and most, if not all, the properties of Russia sheet-iron; and I do hereby declare the following to be a full and exact description of my said process.

The iron is first rolled into sheets in the usual way, leaving them, however, much thicker than they are to be left when finished. The scale which always forms in such cases is then to be removed in the usual manner.

Where such removal is effected by the use of an acid-bath, which is the method I prefer, the sheets are to be immersed in a bath of lime-water to remove or neutralize the acid. This part of the process is not now claimed by me as new.

To prevent ill consequences from any remnant of acid still adhering to the iron, I then apply grease, oil, or any other fatty substance, after which I proceed to carbonize the iron in the following manner: After providing an iron plate of the proper dimensions, on which the sheets of iron, as thus prepared, are to rest, I cover its surface with charcoal, either pulverized or in small lumps, or partly pulverized and partly in lumps. These lumps ought not to be larger than about the size of hickory-nuts, and from that down to charcoal-dust. I then sprinkle on a small quantity of marble-dust, which should be finely pulverized, though no serious ill consequence will result from having the grains of marble considerably coarse. The quantity of this marble-dust is quite small in proportion to the charcoal. I prefer not to use more than one-tenth as much in quantity as there is of charcoal, and good results will be produced by the use of a much smaller quantity. The quantity should mainly depend upon the quality of the iron—the better the quality the less marble-dust will be needed. I then lay on a sheet of the prepared iron, then another coating of charcoal and marble-dust, sufficient to cover the sheet of iron, and a little excess will do no essential injury. Another

sheet of iron is then laid on, and so on, alternating each sheet with a layer of the charcoal and marble-dust, until a sufficient number of sheets has been thus laid on, which will only be limited by the wishes of the operator or the size of the furnace in which they are afterward to be placed. The whole is then placed in the carbonizing-furnace and heated till the iron is brought to a dark-red heat, or a little higher, depending upon the hardness and quality of the iron—the poorer and harder the iron the greater the heat required for this purpose.

The sheets of iron should be allowed to remain in the carbonizing-furnace from fifteen minutes to several hours, according to the thickness of the sheets and the hardness of the iron—the thicker and harder the longer time will be necessary.

This carbonizing may be done before the sheets are immersed in the acid-bath, or they may be immersed in this bath both before and after they have been so carbonized.

The sheets of iron, having thus been prepared, are then heated to a dull-red heat, about to the same degree as in the rolling of ordinary sheet-iron, and they are rolled in the same manner.

At first these sheets are rolled singly. Afterward two sheets are placed together, raised to the degree of heat above described, and then rolled a second time. Then four sheets are placed together, heated, and rolled, and thus, by doubling their number, heating, and rolling them, the sheets can be brought to any desired thickness, the heat in all cases being raised to the degree above intimated, and the rolling should be continued until the sheets are cooled to a black heat. The longer the rolling is thus continued while the sheets are cooling the higher will be the polish given to the iron.

After bringing the sheets to the desired thickness and giving them the requisite polish, they are to be inserted in a furnace or other proper place for being heated in packs and brought to a bright-red heat, for the purpose of annealing and coloring the iron. The sheets are then passed again through the rollers in packs, for a single time, when at a bright-red heat. If not sufficiently annealed,

which the skillful workman will readily perceive, the sheets are then again placed in packs in the annealing box or furnace, and heated gradually to a bright-red heat, and then allowed to cool slowly.

This cooling operation, to be most successful, should continue for several hours, the longer the better. The work is then complete.

The above is the process from which I have obtained the best results; but I do not limit myself to the precise method so described, as it may be considerably varied in many of its parts without seriously impairing the general result; nor do I claim all the parts of the process thus described, when taken respectively by themselves, as some of them are already known; but

What I do claim as new, and desire to secure by Letters Patent, is—

1. The process of forming what is known as

“Russia sheet-iron,” or that which strongly resembles it and possesses most if not all of its properties, substantially in the manner hereinbefore described and set forth.

2. In the process of forming sheet-iron, the use of marble-dust and charcoal for carbonizing the iron preparatory to its receiving the desired surface, substantially in the manner above shown.

3. In the process of forming sheet-iron, the mode of rolling the sheets singly and afterward in packs, in the manner above described—that is to say, by first heating the sheets and then continuing the rolling till they become of a black heat, and even afterward, substantially in the manner above described.

GEORGE ATKINS.

Witnesses:

J. F. CALLAN,  
JULIUS HIRSCH.